

# UNITED STATES PATENT OFFICE.

LUDWIG HERMANN PHILIPPI, OF HAMBURG, GERMANY.

## METHOD OF PRODUCING PHOTO-RILIEVOS.

SPECIFICATION forming part of Letters Patent No. 321,244, dated June 30, 1885.

Application filed January 8, 1883. (No specimens.) Patented in Italy October 4, 1882, No. 16/14636, and in Belgium October 16, 1882, No. 59,109.

*To all whom it may concern:*

Be it known that I, LUDWIG HERMANN PHILIPPI, a subject of the Emperor of Germany, and a resident of Hamburg, in the German Empire, have invented certain new and useful Improvements in Producing Photo-Rilievos with equally deepened excavations, of which the following is a specification.

My invention relates to improvements in photo-rilievos which are produced by etching; and the object of my improvements is to etch the figures of such rilievos to a uniform and equal depth. To attain this object I cover a plate, made of any suitable material that will not be affected or corroded by the etching-acid, with a layer of the material to be etched, such layer being spread equally over the plate and of a uniform thickness. Then I cover the layer with a protecting-couch of etching-varnish, gelatine, printing-ink, &c., which is afterward removed at all the places where the layer is to be etched, or a photographic picture or design may be formed upon the surface of the plate in the usual manner of forming photo-engravings. When a plate thus prepared is exposed to the etching-acid, the upper layer will be eaten away at all the points that are not covered by the protecting-couch; but the excavations thus produced cannot go

farther down or penetrate farther than the 30 non-corrosive base.

Having thus fully described my invention, I claim and desire to secure by Letters Patent—

1. The process of producing photo-rilievo engravings having depressions of equal depth 35 upon their surface, which consists of covering a plate of non-corrosive material with a uniform layer of corrosible material, forming the design upon the said corrosible material in non-corrosive varnish, and etching away 40 the exposed portions of the corrosible material down to the non-corrosive plate, substantially as set forth.

2. A photo-rilievo engraving as produced by the hereinbefore described process, consisting 45 of a uniform layer of corrosible material in combination with a non-corrosive base-plate, so that the depressions etched through the said corrosible material are of equal depth all over the plate, substantially as set forth.

In testimony that I claim the foregoing as my invention I have signed my name, in presence of two witnesses, this 11th day of December, 1882.

LUDWIG HERMANN PHILIPPI.

Witnesses:

ALEXANDER SPECHT,  
EMIL HAASE.